

## UNITED STATES PATENT OFFICE.

FREDERICK M. RUSCHHAUPT, OF MILWAUKEE, WISCONSIN.

## COMPOSITION OF MATTER FOR MANUFACTURING SLATES OR OTHER COVERINGS.

SPECIFICATION forming part of Letters Patent No. 761,788, dated June 7, 1904.

Application filed December 26, 1902. Serial No. 136,738. (No specimens.)

*To all whom it may concern:*

Be it known that I, FREDERICK M. RUSCHHAUPT, a citizen of the United States of America, residing at Milwaukee, in the county of Milwaukee and State of Wisconsin, have invented certain new and useful Improvements in Compositions of Matter for Manufacturing Slates or other Coverings, of which the following is a description.

10 This invention relates to a covering material adapted to serve as a substitute for shingles and slates for roofing or for other covering purposes.

The object of this invention is to produce a 15 covering that will serve as a substitute for shingles and slates for roofing or for other covering purposes by an improved method from a new composition of matter, advisably to be combined with a meshed binder fabric.

20 This object I attain by producing a composition of matter having the desired qualities for a roofing or other covering material, as hereinafter described, by combining the matter produced advisably with a meshed binder fabric, such as wire-netting or other meshed fabric formed advisably of flexible material, 25 in a peculiar and novel manner, as herein-after described.

The composition of matter used in producing the new covering consists of the following ingredients combined substantially in the proportions stated—viz., gum-asphalt, five pounds; asphaltic tar or oil, (so-called "maltha" or "liquid bitumin,") four pounds; clay, 35 (well dried and pulverized or carbonate of lime pulverized,) fifty pounds; fine sand, twenty-five pounds; soapstone or talc, (pulverized and preferably the fibrous variety,) ten pounds; inorganic or organic fibrous material, four 40 pounds, (the inorganic material may be a material like asbestos and the organic material may be a material like wood-pulp or vegetable fiber;) resinate of aluminium, two pounds.

The above ingredients are to be thoroughly 45 mingled by proper agitation in a heating-kettle or other mixing apparatus subjected to a heat of not over 250° Fahrenheit. Care must be taken that the temperature does not overreach 250° Fahrenheit in order that the 50 asphaltic or tarry products will not be decom-

posed. As soon as the mixture or composition in its heating and mixing apparatus assumes a uniform state and while heated it is rolled or otherwise formed into sheets.

When to be used as a substitute for shingles or slates, a meshed fabric, preferably having four to eight meshes to the inch, is employed, onto which two of the sheets of the composition before mentioned are pressed or rolled, one sheet lying on either side of the 55 fabric. It has been found desirable to pass the fabric and inclosing sheets of the composition between two heavy rollers. In this manner the two sheets of composition are forced together with the wire between forming a sheet of the composition having a binder 60 of the meshed fabric at its center. The apparatus, including the rollers, may be of any desired construction, and the rollers will preferably be set apart, so as to form a sheet of 65 about the same thickness as roofing-slates in ordinary use. In consequence of the heavy pressure produced by the rolling process and on account of the limited movability of the ingredients composing the doughy composition the 70 fibrous and integral solid particles or ingredients of the composition will lodge in the mass 75 in accordance with their size, specific gravity, flexibility, and resistance, the ingredients having the greatest specific gravity and some of the 80 fibrous ingredients going to the center of the composite article—viz., the binder fabric and adjacent portions of the two sheets of composition and in this manner the heavier ingredients and some of the fibrous ingredients are 85 entangled with the binder fabric. Thus the coarser parts of the composition are forced to the center of the composite sheet and the finer parts remain near the outside or surfaces 90 of the sheet. After the composite sheet has thus been formed by rolling or pressing two sheets of the composition onto the binder fabric it is passed between a pair of polishing-rollers, which will bring the plate or sheet to the exact thickness desired. The polishing- 95 rollers must be kept constantly moist in order to prevent sticking of the adhesive particles of the composition to their surfaces and in order that the smoothness of the surfaces of the sheet or plate may be attained. The as-

phalt and asphaltic tar aided by the aluminic resinate impart to the composition considerable plasticity while it is warm, and while in a warm state the sheets or plates may easily 5 be embossed or provided with relief-figures for ornamentation. After the composite sheets or plates are formed and polished and while warm they are cut into the desired lengths and sizes and, if desired, may be provided with 10 nail-holes.

Although the ingredients of the composition in their natural state have the qualities desired in the composition, still it is mainly the gum-asphalt and asphaltic oil or tar which 15 impart to the composition its quality of durability and causes it to resist the action of those things and influences to which roofing material is subjected. To produce substitute shingles or slates of different grades, sizes, 20 and qualities different grades of binder fabric may be used. One or more of the ingredients may be omitted, and, in fact, any of the ingredients with the exception of the asphalts. The sand or its equivalent, the clay or talc, 25 and even the meshed binder fabric may be omitted and still a substitute for slate or shingles be produced by combining the remaining ingredients in the proper proportions. It is preferable, however, to use the composition 30 in combination with the binder fabric.

After the finished plates have been produced and have become cold and hard they can by applying heat be rendered sufficiently soft to be capable of being readily cut into pieces of 35 the desired shape or form and also sufficiently soft to be easily folded or bent, so as to conform to angles or curves or valleys on the roofs to which they are applied.

Substitute shingles or slates formed in the manner above set forth resist all action of the 40 weather whether dry or wet, hot or cold, and they will to a great extent resist the influence of a fire in close proximity to them, as they are not easily ignited by sparks, glowing coals, or burning splinters. 45

I am aware that asphaltum and one or another of the ingredients included in my composition have been used for roofing purposes; but I am not aware that all of them have been used in combination or any of them in a substantially similar manner in combination with a meshed binder fabric.

What I claim as my invention is—

1. The herein-described composition of matter, consisting of gum-asphalt, asphaltic oil, 55 sand, clay, talc, fibrous material, and resinate of aluminium.

2. The herein-described composition of matter consisting of gum-asphalt, asphaltic oil, sand, clay, soapstone, or talc, fibrous material, and a resinate insoluble in water. 60

3. A covering material compressed and adhering in sheets, consisting of a composition of gum-asphalt, asphaltic oil, sand, clay, talc and resinate of aluminium, as set forth. 65

4. A sheet of covering material produced under pressure and consisting of a composition of gum-asphalt, asphaltic oil, sand, clay, talc and resinate of aluminium in the proportions stated. 70

In testimony whereof I affix my signature in presence of two witnesses.

FREDERICK M. RUSCHHAUPT.

Witnesses:

JNO. S. GREEN,

HALBERT C. CARTER.